

## UNITED STATES PATENT OFFICE.

ALEXANDER NYMAN, OF NEW YORK, N. Y., ASSIGNOR TO DUBILIER CONDENSER CORPORATION, OF NEW YORK, N. Y., A CORPORATION OF DELAWARE.

## BERYLLIUM FILAMENT.

No Drawing. Application filed November 7, 1924, Serial No. 748,464. Renewed March 4, 1926.

This invention relates to an improved electrical conductor or filament; especially a filament for the emission of electrons.

An object of this invention is to provide a filament preferably of the type utilized in thermionic valves or vacuum tubes of such a character as to afford a relatively large output and high activity, with a comparatively small expenditure of power, and capable of greater durability in service.

The nature of this invention is fully disclosed in the following description; but I, of course, may resort to changes in details to the full extent consistent with the broad and general meanings of the terms in which the appended claim are expressed.

An electrode or filament according to this invention, is made of the chemical element beryllium, which belongs to the alkaline earth group of chemical elements such as barium, strontium and caesium. All of these substances emit electrons freely even at low temperatures, and barium and strontium are extensively used in the form of oxides for coating the filaments of vacuum tubes, in order to afford the emission of electrons at relatively low temperatures of the filament, and with a small consumption of electrical current passing through the filament.

It is known that the melting point of beryllium is quite high, 1280 degrees C., which is higher than the melting point of other alkaline earth elements, and in other ways this element is admirably adapted to withstand conditions to which operation in a vacuum tube connected to a radio circuit, for instance, will expose it.

In accordance with my invention a beryllium filament can be made in various ways, as beryllium is quite ductile and no more

oxidizable than aluminum. A piece of beryllium, therefore, can be easily drawn into wire of the required fineness, and such a filament needs no oxide coating. When mounted in a vacuum tube it will produce electrons in the quantity required, with relatively low current, to the same extent as filaments with oxides or the like on their exterior surfaces.

The resulting filament is quite emissive, very durable, and will operate with comparatively little electrical power and at a low temperature, besides being quite inexpensive to produce.

In practice, I can utilize commercial beryllium which is, of course, impure, and may not contain more than 75% of beryllium, the remaining ingredients being of a different nature and imparting no emissivity. Such commercial beryllium, however, is quite suitable for my purpose, and contains enough of the beryllium to make a cheap filament having the properties above-mentioned, with a high melting point, sufficient ductility and durability, and requiring no oxide coating; while at the same time, having a capacity to emit electrons in large quantity with little electrical power and a low temperature of operation.

Having described my invention, what I believe to be new and desire to secure and protect by Letters Patent of the United States is:—

A filament for emitting electrons, said filament consisting essentially of beryllium.

Signed at New York city in the county of New York and State of New York this 6th day of November, A. D. 1924.

ALEXANDER NYMAN.